

# UNITED STATES PATENT OFFICE.

ARTHUR LINZ, OF NEW YORK, N. Y., ASSIGNOR TO THE CHEMICAL FOUNDATION  
INCORPORATED.

## METHOD OF DYEING.

1,414,029.

Specification of Letters Patent. Patented Apr. 25, 1922.

No Drawing. Original application filed September 1, 1921, Serial No. 497,706. Divided and this application filed December 15, 1921. Serial No. 522,462.

To all whom it may concern:

Be it known that I, ARTHUR LINZ, a citizen of the United States, and a resident of the borough of Manhattan, city, county, and 5 State of New York, have invented an Improvement in Methods of Dyeing, of which the following is a specification.

My invention relates to an improved method of dyeing and has as an object the 10 obtainment of more permanent and fast to light dyeings upon various materials, whereas such dyeings heretofore have been of a relatively fugitive and unstable character.

In my copending application, Serial No. 15 497,706, filed September 1, 1921, there is set forth a method of dyeing which comprises treating the material to be dyed in a solution containing dyestuff, and then subjecting the dyed material to an after treatment 20 in a solution containing a soluble compound of phosphorous and a soluble compound of a difficultly fusible metal, out of which the invention described herein has been divided.

When various materials, such as for example, textiles, leather, hides, and so on, are dyed by the ordinary method, the colors are not always permanent and are sometimes affected by the light. It is an object of my improved method to obviate these possible 25 objections and it is shown that when textiles, leather, and so on, are treated in accordance with my method, the colors obtained thereon are relatively faster and more permanent.

The dyeings hereinbefore referred to depend upon the formation of color lakes and the previous processes for producing these lakes upon various materials are not of such a character as to permit of their general 30 adoption, for the reason that these processes are expensive in consequence of the chemicals employed therein, which chemicals may be produced only through the expenditure of considerable time and labor.

The color lake formation upon textiles, and so forth, has been accomplished through the employment of complex acids containing tungsten, such as for instance, phosphotungstic acid and silicotungstic acid or salts 45 of these complex acids. The preparation of the complex acids or the salts thereof with the attendant separation of the same from the by-products, is an involved, difficult and

expensive procedure, and accordingly their use has materially affected dyeings dependent upon the formation of the color lakes produced through the intermediation of such complex acids or their salts. 55

I have discovered a procedure for the dyeing of textiles, leather, and so on, through the formation of color lakes produced through the use of compounds containing phosphorus and silicon, which shall, during the procedure, interact with compounds containing a difficultly fusible metal, which procedure does not involve the production and isolation of complex acids of difficultly fusible metals or salts of difficultly fusible metals and hence accomplishes a saving of all the expense incident thereto. 60

Further, in consequence thereof my process presents a mode whereby color lakes may be generally applied in dyeing the various materials and at a cost which will admit of their general use and application. 65

The process according to my invention comprises treating textiles, leather, and so on, properly mordanted with compounds containing phosphorus and silicon together with compounds containing a difficultly fusible metal, of which compounds various ones may be used such as, for instance, the acids, that is phosphoric or silicic or their salts, and compounds of such metals as tungsten or molybdenum, and subsequently subjecting the thus treated materials with a solution containing the dye-stuff in the usual manner in accordance therewith, it has been ascertained that such dyeings of textiles, leather and so on are relatively permanent. 70

The following example will serve as an illustrative embodiment of a manner in which my process may be carried into practical effect:

Take a quantity of textile, leather, hides, 75 skins or the like, (for example one hundred pounds) properly mordanted with tannic acid and an antimony salt, or tannin bearing extract and treat the same in a suitable immersion receptacle with a solution in which has been dissolved a phosphate of sodium, e. g., di-sodium phosphate, and sodium tungstate, or a phosphate of sodium and sodium molybdate together with an acid, such as for example, acetic acid to produce in this solution either sodium phosphotungstate, or 80 85 90 95 100 105

phosphotungstic acid, or sodium phosphomolybdate, or phosphomolybdic acid. The above salts may be added in an amount sufficient to produce about five pounds of the complex salt or its equivalent.

After a sufficient incorporation of the salt solution, this solution is displaced by a dye solution containing, for example, about one-half pound of methyl violet. This subsequent treatment may be carried out in the usual manner, either in a vat or a drum and may take place at ordinary temperature, although it may be considered preferable to carry out the subsequent treatment at a raised temperature of say about 70° C.

When it is desired to employ salts of an acid of phosphorus or silicon, together with salts of a difficultly fusible metal, it may be found preferable to add to the dyeing bath a suitable organic or inorganic acid which acid shall be capable of freeing phosphoric, tungstic, molybdic and silicic acids from their respective salts, for which purpose there may preferably be used hydrochloric acid, sulphuric acid and acetic acid which will not affect the coloring matter being used, and it will be understood, of course, that such acid may be entirely dispensed with if the formation of the color lake takes place satisfactorily without its use, and this may be readily determined by simple treatment.

The dyestuffs which may be preferably utilized in my process are usually designated as the basic coal tar dyes and in addition to methyl violet set forth in the above example, there may be employed such dyestuffs as auramine, phosphin, chrysoidin, Bismarck brown, malachite green, emerald green, methylene blue, Victoria blue, crystal violet, saffranine and basic fuchsin, but it will be understood that my process is not limited to the specific class or the specific dyes herein-mentioned, but may be employed for such dyes as will give a permanent and fast color through fixation by means of the compounds set forth.

I claim:

1. The process of dyeing textiles, leather, and so on, which comprises treating said materials with a solution which has been prepared from a soluble compound of phosphorus and a soluble compound of a difficultly fusible metal, and then dyeing said material in the usual manner. 50 55

2. The process of dyeing textiles, leather, and so on, which comprises treating said materials with a solution which has been prepared from a soluble compound of phosphorus and a soluble compound of a difficultly fusible metal and an acid capable of freeing the acid from such compound, and then dyeing said material in the usual manner. 60

3. The process of dyeing textiles, leather, and so on, which comprises treating said material with a solution which has been prepared from a soluble compound of phosphorus and a soluble compound of tungsten, and then dyeing said material in the usual 70 manner. 65

4. The process of dyeing textiles, leather, and so on, which comprises treating said materials with a solution which has been prepared from a phosphate of sodium and tungstate of sodium, and then dyeing said material in the usual manner. 75

5. The process of dyeing textiles, leather, and so on, which comprises treating said materials with a solution which has been prepared from di-sodium phosphate and sodium tungstate, and then dyeing said material in the usual manner. 80 85

6. The process of dyeing textiles, leather, and so on, which comprises treating said materials with a solution which has been prepared from a soluble compound of phosphorus and a soluble compound of a difficultly fusible metal and acetic acid, and then dyeing said material in the usual manner. 90 95

In testimony whereof, I have signed my name to this specification this 9th day of December, 1921.

ARTHUR LINZ.